

No. 669,763.

Patented Mar. 12, 1901.

P. PERRET.

COMPENSATION WATCH BALANCE AND HAIR SPRING.

(Application filed Nov. 26, 1897.)

(No Model.)



Witnesses:

J. A. Blinn  
Peter H. Ross

Inventor:

Paul Perret  
by Henry Comets  
Attorney

# UNITED STATES PATENT OFFICE.

PAUL PERRET, OF CHAUX-DE-FONDS, SWITZERLAND.

## COMPENSATION WATCH BALANCE AND HAIR SPRING.

SPECIFICATION forming part of Letters Patent No. 669,763, dated March 12, 1901.

Application filed November 26, 1897. Serial No. 659,880. (No model.)

*To all whom it may concern:*

Be it known that I, PAUL PERRET, manufacturer, a citizen of the Swiss Republic, residing at Chaux-de-Fonds, Switzerland, have invented certain new and useful Improvements 5 in Escapements for Watches, Clocks, and the Like, (which have been patented in Switzerland by Letters Patent No. 14,270, dated May 6, 1897,) of which the following is a specification.

This invention relates to improvements in all kinds of escapements for watches, clocks, and the like; and it consists, mainly, in the combination of a balance or hair spring made 15 of an alloy formed of about seventy-two parts, by weight, of steel and about twenty-eight parts, by weight, of nickel, with an ordinary balance—that is to say, a non-compensation balance—made of brass. The increase 20 in elastic force of the balance-spring formed of this alloy with the rise of temperature is just sufficient to compensate for the increase of the moment of inertia of the balance due to its expansion.

25 In the accompanying drawing I have shown an ordinary or non-compensation balance adapted to operate in connection with my improved balance-spring.

In the drawing, *a* designates the balance-spring, and *b* is the balance-wheel, made of 30 brass.

In this specification the term "nickel" signifies commercial nickel and not chemically-pure metal, and the term "brass" signifies all alloys of copper which have nearly the 35 same coefficient of expansion as the usual brass.

What I claim is—

The combination of a non-compensation balance made of brass, with a balance-spring 40 of the usual form made of an alloy formed of about seventy-two parts by weight of steel and about twenty-eight parts by weight of nickel and having the property of increasing its elastic force with a rise of temperature 45 just sufficiently for obtaining a compensation for the expansion of the uncompensated balance.

In witness whereof I have hereunto signed my name in the presence of two subscribing 50 witnesses.

PAUL PERRET.

Witnesses:

ARMAND FERRELET,  
EPHRIAM HUGUENIN.